

## UNITED STATES PATENT OFFICE

2,678,881

## CORROSION RESISTANT ALLOY

William O. Binder and Claude R. Bishop, Niagara Falls, N. Y., assignors to Union Carbide and Carbon Corporation, a corporation of New York

No Drawing. Application December 10, 1949,  
Serial No. 132,426

4 Claims. (Cl. 75—122)

1

This invention relates to iron-nickel-molybdenum alloys and refers more particularly to alloys of this type containing antimony and possessing excellent resistance to corrosion by reducing acids together with good machinability.

Nickel-base alloys containing about 10% to 40% molybdenum and a small proportion of iron, generally not exceeding about 5% to 20% have enjoyed rather widespread use for many years by reason of their excellent resistance to corrosion in reducing acid media such as hot concentrated hydrochloric acid. However, a disadvantage of these alloys is their rather high cost which is due in part to their high content of expensive nickel and molybdenum and in part to the difficulty which is encountered in machining them, which difficulty raises fabrication costs.

It is the principal object of this invention to provide iron-nickel-molybdenum alloys which combine the excellent corrosion resistance of the prior alloys with greater machinability and a lower proportion of expensive constituents.

This object is achieved by the invention which is an alloy containing 30% to 70% iron; 1% to 25% molybdenum; 0.25% to 3% antimony; the

and the remainder nickel and incidental impurities, the nickel content being at least 45%.

Although in the past it has been considered that raising the iron content of prior nickel-molybdenum-iron alloys seriously detrimentally affects corrosion resistance and therefore that the iron content of such alloys should in no event exceed 25%, in the present invention iron is substituted for molybdenum and nickel without undue loss of corrosion resistance provided antimony is present in the specified proportions. Many corrosion tests have demonstrated that the alloy of the present invention possesses corrosion resistance at least equivalent to that of the prior alloys in the same media.

In the following table typical results of corrosion tests conducted on samples which were sand cast, heated 1/2 hour at 1100° C. and air cooled are set forth. In these tests the samples were weighed, immersed in boiling 10% hydrochloric acid for 48 hours, removed, washed and weighed and again immersed for 48 hours in the boiling acid. Each sample was thus tested for five 48 hour periods and the corrosion rate calculated and reported as inches penetration per month.

Table I

| Percent Composition;<br>Remainder Ni |    |     |       | Corrosion Rate, Inch Penetration per Month |               |              |               |              |         |
|--------------------------------------|----|-----|-------|--------------------------------------------|---------------|--------------|---------------|--------------|---------|
| Mo                                   | Fe | Sb  | C     | First Period                               | Second Period | Third Period | Fourth Period | Fifth Period | Average |
| 29                                   | 5  | Nil | 0.053 | 0.00113                                    | 0.00095       | 0.00145      | 0.0024        | 0.0017       | 0.00153 |
| 20                                   | 20 | Nil | 0.039 | 0.018                                      | 0.037         | 0.043        | 0.061         | 0.067        | 0.045   |
| 1                                    | 40 | 2   | 0.006 | 0.0165                                     | 0.00205       | 0.0035       | 0.0049        | 0.0126       | 0.0070  |
| 3                                    | 40 | 2   | 0.009 | 0.0145                                     | 0.0073        | 0.00024      | 0.0047        | 0.00049      | 0.0043  |
| 5                                    | 30 | 2   | 0.015 | 0.0166                                     | 0.0016        | 0.00105      | 0.00142       | 0.00124      | 0.0014  |
| 5                                    | 40 | 2   | 0.01  | 0.0028                                     | 0.00085       | 0.00075      | 0.00040       | 0.00070      | 0.0011  |
| 5                                    | 60 | 2   | 0.011 | 0.0043                                     | 0.0093        | 0.00112      | 0.00071       | 0.00090      | 0.0033  |
| 10                                   | 40 | 2   | 0.021 | 0.0018                                     | 0.00107       | 0.0014       | 0.0012        | 0.0012       | 0.0013  |
| 15                                   | 30 | 2   | 0.025 | 0.00072                                    | 0.00053       | 0.00035      | 0.00116       | 0.00125      | 0.00080 |
| 15                                   | 40 | 2   | 0.030 | 0.00195                                    | 0.0033        | 0.00048      | 0.00055       | 0.00073      | 0.0014  |
| 15                                   | 50 | 2   | 0.024 | 0.0028                                     | 0.00214       | 0.00252      | 0.00186       | 0.00158      | 0.0021  |
| 20                                   | 35 | 2   | 0.043 | 0.020                                      | 0.00162       | 0.00202      | 0.00274       | 0.00185      | 0.0020  |

remainder nickel and incidental impurities; the nickel content being at least 26%. For severe conditions of service requiring a high degree of corrosion resistance and good ductility, it is preferred that the alloy of the invention contain 30% to 50% iron; 2% to 20% molybdenum; 0.25% to 3% antimony; the remainder nickel and incidental impurities, the nickel content being at least 45%. Up to 5% copper may be added to the alloy with benefit, the copper addition improving resistance of the alloy to boiling dilute sulfuric acid. A particularly preferred range of composition is 4% to 8% molybdenum; 35% to 45% iron; up to 3% copper; 0.5% to 2.5% antimony

In the table above the first two alloys are representative of the prior art and differ from each other in that the second contains less molybdenum and nickel and more iron than the first. It will be observed that the second alloy is much less resistant to the test medium than the first. The remainder of the compositions listed in the table are representative of the alloy of the invention and differ from the first two compositions in that they contain 2% antimony and have increased iron content and decreased molybdenum and nickel contents. It will be observed that each of these compositions exhibited greater average resistance to the test medium than did

the second alloy in the table and compares very favorably with the first alloy in the table, some compositions showing even less attack than the first alloy.

In Table I, it will be noted, the antimony content of the compositions tested was held at 2% while the molybdenum, nickel and iron contents were changed. Another series of tests was made with varying antimony content and results of some of these tests are reported in Table II. The specimens were tested in the same condition of heat treatment as in the tests reported in Table I and the tests were conducted in the same way in boiling 10% hydrochloric acid.

Table II

| Composition: 40% Fe,<br>remainder Ni and |               |                   | Corrosion Rate, Inch penetration per month |                  |                 |                  |                 |         |
|------------------------------------------|---------------|-------------------|--------------------------------------------|------------------|-----------------|------------------|-----------------|---------|
| Percent<br>Mo                            | Percent<br>Sb | Percent<br>C      | First<br>Period                            | Second<br>Period | Third<br>Period | Fourth<br>Period | Fifth<br>Period | Average |
| 5                                        | 0.26          | 0.006             | 0.0037                                     | 0.0242           | 0.059           | 0.077            | 0.108           | 0.054   |
| 5                                        | 0.5           | <sup>1</sup> 0.03 | 0.0016                                     | 0.0034           | 0.0056          | 0.0059           | 0.0079          | 0.0059  |
| 5                                        | 1.02          | 0.027             | 0.00294                                    | 0.00080          | 0.00085         | 0.00060          | 0.00094         | 0.0012  |
| 5                                        | 1.47          | 0.015             | 0.00254                                    | 0.00142          | 0.00090         | 0.00173          | 0.00125         | 0.0016  |
| 5                                        | 2.0           | 0.010             | 0.0028                                     | 0.00085          | 0.00075         | 0.00040          | 0.00070         | 0.0011  |
| 5                                        | 3.0           | 0.017             | 0.00156                                    | 0.00096          | 0.00076         | 0.00078          | 0.00101         | 0.00101 |
| 15                                       | 0.23          | 0.026             | 0.0094                                     | 0.0295           | 0.054           | 0.051            | 0.09            | 0.048   |
| 15                                       | 0.96          | 0.023             | 0.0023                                     | 0.00275          | 0.00242         | 0.0019           | 0.00183         | 0.0022  |
| 15                                       | 1.50          | 0.028             | 0.00111                                    | 0.00105          | 0.0013          | 0.00114          | 0.0014          | 0.0012  |
| 15                                       | 2.0           | 0.03              | 0.00195                                    | 0.0033           | 0.00048         | 0.00055          | 0.00073         | 0.0014  |
| 15                                       | 2.94          | 0.027             | 0.00086                                    | 0.00096          | 0.00111         | 0.00124          | 0.0012          | 0.00107 |

<sup>1</sup> Also contains 2% Cu.

From the data of Table II it is apparent that for maximum corrosion resistance more than 0.25% antimony should be present in the alloy of the invention but that raising the antimony content from 2% to 3% gives no substantial added benefit.

The beneficial effect of copper in the alloy of the invention has been demonstrated by tests in boiling 10% sulfuric acid. For example an alloy containing 5% molybdenum; 40% iron; 2% antimony; 0.01% carbon; remainder nickel showed an average (three 48 hour periods) corrosion rate of 0.0078 inch penetration per month, whereas the corrosion rate of an alloy exactly similar except that it contained 2% copper (replacing 2% nickel) and 0.016% carbon showed an average (three 48 hour periods) corrosion rate of 0.00033 inch penetration per month in the same medium.

Tensile tests of the alloy of the invention have shown it to possess useful strength and ductility but indicate that for maximum strength and ductility the antimony content should not exceed 2%. More than 3% antimony tends to cause excessive brittleness. The ductility of compositions containing not more than 2% antimony generally is greater than that of prior alloys free of antimony, as evidenced by elongation of tensile test specimens.

Although antimony of itself apparently has little effect on the machinability of the alloy of the invention the alloy is significantly improved in machinability as compared to prior nickel-molybdenum-iron alloys presumably because of the present alloy's increased iron content and lower molybdenum and nickel contents. Comparative machinability tests were made by machining cast samples of different compositions in conventional manner with conventional tools. The machining tests were continued on the conventional nickel-molybdenum-iron alloys until the cutting edge of the tool failed. The diameter of the specimen multiplied by the length of cut (expressed as "D. L.") is a measure of the ma-

chinability of the specimen. These tests indicate that the alloy of the invention has machinability of at least three times as great as that of conventional nickel-molybdenum-iron alloys. Furthermore the cutting edge of the tool showed no evidence of failure during the period of test on the alloy of the invention.

As is true of ferrous alloys in general, carbon is an unavoidable impurity in the alloy of the invention. Care should be taken that the carbon content be as low as possible. In accordance with good alloy-making practice, the alloy of the invention is deoxidized, conveniently with manganese and silicon, and the finished alloy may con-

tain as impurities residual quantities of the deoxidizers used.

The alloys of the invention should be annealed after casting for optimum corrosion resistance. A satisfactory annealing heat treatment consists of heating the alloy about  $\frac{1}{2}$  hour at 1100° C. and air cooling. The cooling rate should be rapid enough to retain substantially the elevated temperature structure produced by annealing.

We claim:

1. An alloy containing 30% to 70% iron; 1% to 25% molybdenum; 0.25% to 3% antimony; up to 5% copper; the remainder nickel and incidental impurities, the nickel content being at least 26%.

2. An alloy containing 30% to 50% iron; 2% to 20% molybdenum; 0.25% to 3% antimony; up to 5% copper; the remainder nickel and incidental impurities, the nickel content being at least 45%.

3. A corrosion-resistant alloy containing 4% to 8% molybdenum; 35% to 45% iron; up to 3% copper; 0.5% to 2.5% antimony; the remainder nickel and incidental impurities, the nickel content being at least 45%.

4. A cast article required in its normal use to withstand corrosion by reducing acids, said article being composed of the alloy defined by claim 1.

#### References Cited in the file of this patent

#### UNITED STATES PATENTS

| Number    | Name     | Date           |
|-----------|----------|----------------|
| 1,939,890 | Frischer | Dec. 19, 1933  |
| 2,054,927 | Carius   | Sept. 22, 1936 |
| 2,219,445 | Franks   | Oct. 29, 1940  |
| 2,222,473 | Bishop   | Nov. 19, 1940  |
| 2,334,870 | Franks   | Nov. 23, 1943  |

#### FOREIGN PATENTS

| Number | Country | Date                                  |
|--------|---------|---------------------------------------|
| 47,686 | France  | Mar. 9, 1937<br>(Addition to 791,803) |